

## UNITED STATES PATENT OFFICE

2,061,264

## PROCESS OF RECONDITIONING METAL ARTICLES

Lawrence S. Wilbur, Evanston, Ill.

No Drawing. Application February 10, 1934,  
Serial No. 710,660

## 5 Claims. (Cl. 148—12)

This invention relates to the reconditioning of worn metal articles to render them suitable for reuse.

More specifically, this invention relates to a process for restoring worn splice bars that have been used for joining railroad rails.

While the process of this invention is applicable to the reconditioning of any worn shaped metal article, it is particularly adapted to the reconditioning of ferrous metal articles and has particular utility in the reshaping, reclaiming and restoring of railroad splice bars. For the sake of convenience, the invention will hereafter be described as embodied in the preferred form 15 applied to railroad splice bars.

It is readily appreciated that splice bars in use at the junction of railroad rails are subjected to various conditions that induce wear to such an extent as to render them unfit for service after 20 a period of time. These worn splice bars must be replaced by new bars or subjected to a reconditioning treatment to make them again serviceable.

Most of the splice bars now in use are made 25 of heat-treated, high carbon steel, and it is with such material that the process of this invention is particularly applicable. Generally, the splice bars have a carbon range of from .3% to .7% and a tensile strength before heating approximating 85,000 pounds per square inch. After heat-treatment, the tensile strength is increased to around 125,000 pounds per square inch.

In the manufacture of new splice bars, the steel mills have an accurate analysis of each 35 batch made so that the proper heat-treatment may be given to the batch to bring the bars to the desired tensile strength. Although the different batches may vary considerably in carbon content within the range indicated above, the 40 heat-treatment is controlled for each batch to produce the same final tensile strength for all batches. Thus the finished bars from various batches will vary widely in carbon content but will all have a tensile strength of approximately 45 110,000-130,000 pounds per square inch.

When the bars have been placed into service and are removed because of wear or for other reasons, they are hopelessly mixed as to carbon content, so that the carbon content of any single 50 bar or any group of bars is unknown. It would be necessary to analyze each individual bar in any group for its carbon content so that the proper heat treatment could be given to the bars to bring them to the uniform tensile strength 55 which they possessed when newly made. It is

obvious that the cost and time involved in analyzing each individual bar would defeat any reconditioning process, from a commercial standpoint.

The purpose of my invention is to provide a process whereby the bars are considerably equalized so that they may all undergo the identical reconditioning steps and possess satisfactory tensile strength and ductility to pass the specification tests. 5

It is therefore an object of this invention to provide an economical process for reconditioning worn metal objects.

Another object of this invention is to provide a reconditioning process for worn metal objects that is applicable to ferrous metals of unlike carbon contents to yield reconditioned articles of 15 similar physical characteristics.

Another object of this invention is to provide a heat treating process for worn splice bars that will change the steel structure of the bars so that 20 the treated bars will be superior to the new bars.

Another object of this invention is to relieve the strains set up in splice bars during their use in railroad tracks.

A specific object of this invention is to provide 25 an economical reconditioning process that is applicable to batches of splice bars having unknown carbon contents to produce reconditioned bars having similar tensile strength and bending properties.

Other and further objects of this invention will 30 be apparent to those skilled in the art from the following specification.

The process of my invention will now be described as applied to a batch of worn-out splice 35 bars formed of steel having a carbon content of .3% and .7%, which steel has been heat-treated to have a tensile strength of approximately 125,000 pounds per square inch. These worn-out bars most probably have been subjected to years 40 of service and are cracked, bent, warped, rusted and strained. It will be appreciated that the carbon content of each individual bar is unknown, except that it is within the range above indicated because railroad specifications call for the use of 45 steel having this carbon range.

The worn bars are first placed in an annealing furnace and heated to temperatures above the point of "decalescence" or upper critical  $A_{c1}$  point. 50 These temperatures, for steels of the grades indicated, are between 1600 to 1800° F.

The heated bars are then removed from the furnace and stacked together in piles so that they may cool slowly in the air. This step of the proc- 55

ess is called a normalizing step and is practiced to relieve strains set up in the bars during usage. The cooled, normalized bars are next placed in a furnace and heated to a forging temperature, preferably between 1450 to 1800 degrees F. The heated bars, at the temperature indicated, are removed from the furnace one at a time, and placed between re-forming dies where they are re-shaped under pressure applied to the bars. 10 The pressure causes the metal of the bars to flow into the recesses of the dies so that the bars are re-formed to the desired dimensions.

The pressed bars are next subjected to a quenching operation to harden the steel. The 15 quenching material may be any type of well-known quenching oil, water or any suitable quenching medium. The quench, however, must be severe enough to cause the bars having a lower carbon content (bars of .3% carbon) to attain a 20 tensile strength above 100,000 pounds per square inch, preferably approximately 110,000 pounds per square inch. This severe quench will increase the tensile strength of the higher carbon content bars to approximately 160,000 pounds per square 25 inch.

The re-formed carbon bars having the lower carbon content are satisfactory for use, because they possess a suitable tensile strength and, also, are ductile enough to pass the required bend test. 30 Railroad specifications require that splice bars must not fail when bended, cold, to a 45 degree angle. However, the splice bars formed of higher carbon steel are too brittle to pass the bend test and it is therefore necessary to reduce the brittleness 35 of the higher carbon bars. This must be accomplished without materially lowering the tensile strength of the lower carbon bars. Since the carbon analysis of the bars being treated is not known, it is impossible to segregate the batch 40 so that the brittle bars may be treated alone.

I have found that the malleability and tensile strength of the bars may be considerably equalized by treating the splice bars in a drawing furnace at suitable temperatures for a length of time 45 that will reduce the strain set up in the higher carbon bars during the violent quench treatment, but will not seriously impair the tensile strength of the lower carbon bars.

It is known that high carbon steels that have 50 been quenched to higher tensile strengths are affected much more by a drawing operation than are lower carbon steels with lower tensile strengths. Because of this phenomenon, I am 55 able to bring the extremes of brittleness and tensile strengths of the bars closer together, or, in other words, to equalize the physical characteristics of the batch. For example, a low carbon content bar having a tensile strength of 110,000 pounds per square inch and a high carbon content bar having a tensile strength of 160,000 60 pounds per square inch, when treated in accordance with my invention, in a drawing furnace, can be equalized so that the first bar is only reduced in tensile strength to approximately 100,000 65 pounds per square inch, while the second bar is reduced to about 125,000 pounds per square inch. In this manner, the low tensile strength bar can still pass the railroad specifications for a minimum of 100,000 pounds per square inch tensile 70 strength, while the higher tensile strength bars will have sufficient malleability or ductility to pass the required bend test.

I have found that a given batch of rail bars may thus be equalized by heating in a drawing furnace to temperatures of about 500 to 800° F. 75

for about 30 minutes to two hours. Obviously, this treatment can be varied considerably to fit specific conditions without departing from the principle of this invention.

The normalizing, forging, quenching and drawing operations of this process each cooperates to produce bars having a better grain structure than the new bars. It is well known to metallurgists that the working of a metal benefits its grain structure. 5 10 15

While the above description of my process covers a preferred working operation, it is obvious that some of these steps may be omitted in some instances, and that other auxiliary steps can be included. For example, the normalizing 15 step may be used alone in some instances or may be dispensed with in other instances. The bars may be ground with an abrasive wheel at the center part of the upper bearing surface to search for cracks, or they may be subjected to a cleaning 20 or pickling process to remove rust and dirt. The cleaning operation may be inserted just before the bars are placed in the forming dies. The forming dies may be provided with pins to preserve the holes, or the bars may be repunched, 25 or the holes may be ignored during the re-forming operation.

From the above description it is evident that I have provided a process, including several 30 steps, which may be performed in proper sequence to recondition worn-out splice bars of unknown and mixed carbon contents so that the treated bars will pass the requirements of new bars. As pointed out above, the process is applicable to the reconditioning of other shaped 35 metallic articles.

I am aware that many changes may be made and numerous details of construction may be varied through a wide range without departing from the principles of this invention, and I, 40 therefore, do not purpose limiting the patent granted hereon otherwise than necessitated by the prior art.

I claim as my invention:

1. The process of reconditioning a batch of 45 worn railroad splice bars having unknown carbon contents within the range of 0.3 to 0.7% and having unknown tensile strengths within the range of 110,000 to 160,000 pounds per square inch to produce reformed bars which are sufficiently ductile to pass railroad bend test requirements and having tensile strengths not lower than 100,000 pounds per square inch which comprises heating said bars to temperatures between 50 1600° to 1800° F., allowing the heated bars to cool slowly, reheating said cooled bars to forging temperatures between 1450° to 1800° F., reforming said bars under pressure at the forging temperatures, quenching the re-formed bars and again reheating the bars to temperatures around 55 600° F.

2. The process of reconditioning a batch of worn out splice bars of unknown carbon contents within the range of 0.3% to 0.7% and unknown tensile strengths within the range of 110,000 to 65 160,000 lbs./sq. in. to produce re-formed splice bars sufficiently ductile to pass railroad bend test requirements and strong enough to pass railroad tensile strength requirements which comprises heating said worn out splice bars to temperatures between 1600 to 1800° F., stacking the heated splice bars in piles in contact with the air, allowing the stacked bars to cool, reheating the bars to temperatures between 1450 and 1800° F., reshaping the reheated bars under die pres- 70 75

- sure, quenching the reshaped bars in a quenching liquid and reheating the quenched bars to temperatures around 600° F. in a drawing furnace.
5. 3. The process of reconditioning a batch of worn railroad splice bars having unknown carbon contents within the range of 0.3 to 0.7% and having unknown tensile strengths within the range of 110,000 to 160,000 pounds per square 10 inch to produce re-formed bars which are sufficiently ductile to pass railroad bend test requirements and having tensile strengths not lower than 100,000 pounds per square inch which comprises heating said splice bars to temperatures 15 between 1450 to 1800° F. in an annealing furnace, stacking the bars in piles in the air, allowing said stacked bars to cool, reheating the cooled bars to temperatures between 1450 to 1800° F., reshaping said heated bars under pressure, 20 quenching the reshaped bars in a quenching medium to increase their tensile strength and subjecting the quenched bars to a drawing operation to temperatures around 600° F. for about 40 minutes to increase their ductility.
25. 4. The process of reconditioning worn splice bars of unknown carbon contents within the range of 0.3% to 0.7% and having unknown tensile strengths within the range of 110,000 to 160,000 lbs./sq. in. to produce re-formed bars

which are sufficiently ductile to pass railroad bend test requirements and having tensile strengths not lower than 100,000 lbs./sq. in. which comprises heating said bars to temperatures between 1600 degrees and 1800 degrees F., 5 allowing the heated bars to cool slowly, reheating the cooled bars to forging temperatures, re-forming the bars under pressure at the forging temperatures, quenching the re-formed bars, and heating the quenched bars to increase their ductility.

5. The process of reconditioning worn splice bars of unknown carbon contents within the range of 0.3% to 0.7% and having unknown tensile strengths within the range of 110,000 to 160,000 lbs./sq. in. to produce re-formed bars which are sufficiently ductile to pass railroad bend test requirements and having tensile strengths not lower than 100,000 lbs./sq. in. 15 which comprises heating said bars to temperatures between 1600 degrees and 1800 degrees F., allowing the heated bars to cool slowly, reheating the cooled bars to temperatures between 1450 degrees and 1800 degrees F., reshaping the heated bars under die pressure, quenching the reshaped 20 bars in a quenching liquid, and reheating the quenched bars in a drawing furnace to increase their ductility.

LAWRENCE S. WILBUR.